# EUROPEAN PATENT SPECIFICATION

(11) **EP 2 034 036 B1**
(45) Date of publication and mention of the grant of the patent: **11.12.2013**
(21) Application number: 08014230.0
(22) Date of filing: 08.08.2008
(51) Int. Cl.: C22C 38/02, C22C 38/04, C21D 8/06, C22C 38/00, C21D 9/52, D07B 1/06, B21C 1/00

(54) **Wire rod having excellent wire drawability and its production method**
Walzdraht mit hervorragender Drahtziehfähigkeit und Herstellungsverfahren dafür
Fil-machine disposant d'une excellente aptitude à l'étirage et son procédé de production

(30) Priority: 05.09.2007 JP 2007230713
(43) Date of publication of application: 11.03.2009
(73) Proprietor: Kabushiki Kaisha Kobe Seiko Sho (Kobe Steel, Ltd.), Kobe-shi, Hyogo 651-8585 (JP)
(72) Inventor: Kochi, Takuya, Kobe-shi, Hyogo 651-2271 (JP); Maruo, Tomotada, Kobe-shi, Hyogo 657-0863 (JP); Nishimura, Masumi, Kagogawa-shi, Hyogo 675-0137 (JP)
(74) Representative: Müller-Boré & Partner Patentanwälte

(56) References cited:
- EP-A1- 0 169 587
- EP-A1- 0 341 680
- EP-A1- 0 708 182
- EP-A1- 1 018 565
- EP-A1- 1 277 846
- EP-A1- 1 674 588
- JP-A- 60 152 659
- JP-A- 2000 219 938
- JP-A- 2000 336 458
- JP-A- 2001 064 753
- US-A- 4 020 887
- US-A1- 2004 129 354
- US-A1- 2006 048 864

## Description

The present invention relates to a wire rod (hot rolled wire rod) which becomes a raw material for wire rod products such as steel cords, bead wires.

Steel cords, bead wires or the like are manufactured usually by wire drawing after descaling (mechanical descaling, acid washing treatment or the like, for example) the wire rod obtained by hot rolling of a billet with approximately 0.7-0.8% carbon content. If the wire rod is broken in wire drawing, productivity is impaired markedly, therefore excellent wire drawability is required for wire rods.

The present applicant previously proposed several techniques for improving wire drawability of wire rods.

In JP-A-2004-137597 (Patent Document 1), a technique is disclosed where drawability is improved in wire drawing of the wire rod in an as-hot-rolled state, in addition to by stipulating the composition of the wire rod, by stipulating the average value of the tensile strength, the standard deviation of the tensile strength, the average value of the fracture drawing, and the standard deviation of the fracture drawing, of the wire rod.

In JP-A-2005-206853 (Patent Document 2), a wire rod is proposed wherein a patenting treatment before or during wire drawing can be omitted and excellent wire drawing is possible in an as-hot-rolled state, in addition to by stipulating the composition of the wire rod, by stipulating the average tensile strength and the average lamellar spacing.

In JP-A-2006-200039 (Patent Document 3), a wire rod is proposed wherein increase of wire drawing speed, increase of reduction ratio of area, and extension of the life time of a dice are possible, in addition to by stipulating the composition of the wire rod, by optimizing the metal structure (average crystal particle diameter and the maximum crystal particle diameter).

However, the wire rod actually proposed in an example level in the Patent Documents contained C by more or less 0.8% to secure the tensile strength of 3,500 MPa level by wire drawing. Consequently, tensile strength of most of wire rods exceeded 1,000 MPa, and wire drawing speed could not be increased and remained at 800 m/min at maximum. (Refer to Patent Document 3.)

On the other hand, in the market, although there is a demand for the wire rods whose tensile strength becomes 3,500 MPa level by wire drawing, a demand of the wire rods whose tensile strength becomes 3,000 MPa level after wire drawing is greater, and at present, the latter wire rods are in circulation as the wire rods for the use of general products. Therefore, the wire rod, whose tensile strength becomes 3,000 MPa level after wire drawing, which does not cause wire breakage even if it is drawn at high speed, and which does not shorten the life time of a dice, is required.

EP 1 674 588 A1 discloses a high carbon steel wire material having excellent wire drawability and manufacturing process thereof.

Under the circumstances the present invention has been developed and its purpose is to provide a wire rod, whose tensile strength after wire drawing becomes more or less 3,000 MPa level, which does not cause wire breakage even if the wire drawing speed is increased, which does not shorten the life time of a dice, and whose wire drawability is improved. Another purpose of the present invention is to provide a method for producing a wire rod excellent in wire drawability.

The wire rod according to claim 1 of the present invention addressing the aforementioned problems is the wire rod with the essential points of consisting of C: 0.65-0.75% (in mass%, hereafter the same with regard to the composition), Si: 0.1-0.5%, Mn: 0.1-0.6%, P: 0.015% or below (not including 0%), S: 0.015% or below (not including 0%), N: 0.004% or below (not including 0%), Al: 0.003% or below (not including 0%), O: 0.003% or below (not including 0%), optionally Cr: 0.5% or below (not including 0%), optionally Cu: 0.5% or below (not including 0%) the balance being iron and inevitable impurities, wherein tensile strength (TS) is 960 MPa or below, and reduction of area (RA) is 40% or above.

The wire rod of the present invention is be produced by going through a process for heating a billet satisfying the above composition at from 1,000 to 1,080 DEG C., a process for hot rolling of the heated billet with the lowest temperature during rolling being made at from 820 to 920 DEG C., a process for finish rolling of the wire rod obtained by the hot rolling at from 900 to 980 DEG C., a process for winding the wire rod obtained by the finish rolling at from 880 to 940 DEG C., a process for cooling the wound wire rod from the winding temperature to 800 DEG C. at average cooling rate (CR₁) of 10 DEG C./s or below, a process for cooling consecutively from 800 DEG C. to the temperature T₁ of 640-600 DEG C. at average cooling rate (CR₂) of 30 DEG C./s or above, and a process for heating the wire rod cooled to the temperature range of 640-600 DEG C. at a temperature T₂ of 680 DEG C. or below, wherein the temperature T₂ exceeds the temperature T₁.

In accordance with the aspects of the present invention, by hot rolling of the billet whose composition is stipulated under an appropriate condition and by subsequently cooling under an appropriate condition, the tensile strength of the wire rod can be made 960 MPa or below and the reduction of area can be made 40% or above, accordingly, the wire drawing speed can be made higher than before in wire drawing of the wire rod, and shortening of the life time of the dice can be avoided.
FIG. 1 is a drawing showing the heat pattern in producing the hot rolled wire rod in accordance with the present invention.
FIG. 2 is a graph showing the relation between tensile strength (TS) and reduction of area (RA).

The present inventors have made intensive investigations to improve wire drawability of the wire rod whose tensile strength becomes 3,000 MPa level in wire drawing. As a result, it was found out that wire rod drawability could be improved if the tensile strength of the hot rolled wire rod was made 960 MPa or below and the reduction of area was made 40% or above, and that, in order to make such tensile strength and reduction of area coexist, the composition of the hot rolled wire rod should be adjusted appropriately and the hot rolling condition and the cooling condition after hot rolling should be controlled appropriately, and the present invention was accomplished.

First, the composition of the hot rolled wire rod in accordance with the present invention will be described. The hot rolled wire rod in accordance with the present invention consists of C: 0.65-0.75%, Si: 0.1-0.5%, Mn: 0.1-0.6%, P: 0.015% or less (not including 0%), S: 0.015% or below (not including 0%), N: 0.004% or below (not including 0%), Al: 0.003% or less (not including 0%), O: 0.003% or less (not including 0%), optionally Cr: 0.5% or below (not including 0%), optionally Cu: 0.5% or below (not including 0%) and the balance being iron and inevitable impurities.

C is the element necessary for securing the strength of wire rod products. However, the purpose of the present invention is to provide the hot rolled wire rod which becomes the raw material of, among wire rod products, not the high strength product whose tensile strength is 3,500 MPa level, but the general product whose tensile strength is 3,000 MPa level. Although C of the hot rolled wire rod is required to be made as much as possible in producing the high strength product, because production of the general product is envisaged in the present invention, C of the hot rolled wire rod is comparatively less than the case of production of high strength product, and is to be in the range of 0.65-0.75%.

However, if C is below 0.65%, tensile strength of wire rod products cannot be secured, therefore, C is made 0.65% or above, preferably 0.68% or above, or more preferably 0.7% or above. On the other hand, if C is contained excessively, wire drawability is deteriorated because tensile strength becomes too high, ductility is deteriorated, and reduction of area becomes little. Therefore, C is made 0.75% or below, preferably 0.74% or below, or more preferably 0.73% or below.

Si is the element acting as a deoxidizing agent. If Si is below 0.1%, deoxidization is not enough, troubles in steel making become liable to occur, and wire drawability of wire rods is deteriorated as solid solution oxygen increases. Therefore, Si is required to be contained by 0.1% or above, preferably 0.13% or above, or more preferably 0.15% or above. On the other hand, Si increases the strength of the hot rolled wire rod by solid solution strengthening and has an action to promote decarburization. However, if Si becomes excessive, the tensile strength of the hot rolled wire rod becomes too high and wire breakage occurs in wire rod drawing. Therefore, Si is made 0.5% or below, preferably 0.48% or below, or more preferably 0.4% or below.

Not only acting as a deoxidizing agent, Mn also has an action to detoxify S by fixing S, a harmful element, as MnS. Also, Mn has an action to stabilize carbide in steel. However, if Mn is below 0.1%, detoxification of S becomes insufficient and drawability of wire rods is deteriorated. Further, crack possibly occurs in hot rolling. Therefore, Mn is required to be contained by 0.1% or above, preferably 0.13% or above, or more preferably 0.2% or above. However, if Mn becomes excessive, the tensile strength of the hot rolled wire rod becomes too high and wire breakage occurs in wire drawing. Also, segregation and super cooled structure are liable to occur which become the cause of wire breakage. Therefore, Mn is made 0.6% or below, preferably 0.58% or below, or more preferably 0.55% or below.

P is an inevitable impurity element, and if it is contained in excess, it deteriorates toughness and ductility of the hot rolled wire rod which becomes the cause of wire breakage in wire drawing. Therefore, P is made 0.015% or below, preferably 0.014% or below, more preferably 0.013% or below, further more preferably 0.010% or below.

S is an inevitable impurity element, is trapped by Mn and is fixed as MnS. However, if S becomes excessive, because MnS amount increases and the size becomes large, ductility of the hot rolled wire rod deteriorates which becomes the cause of wire breakage in wire drawing. Therefore, S is made 0.015% or below, preferably 0.013% or below, more preferably 0.01% or below, further more preferably 0.007% or below.

Although N is an inevitable impurity element, it is an element acting for improving tensile strength of the hot rolled wire rod by age hardening. However, if it is contained in excess, it deteriorates ductility of the hot rolled wire rod which becomes the cause of wire breakage in wire drawing. Therefore, N is made 0.004% or below, preferably 0.0035% or below, more preferably 0.003% or below, further more preferably 0.0025% or below, especially more preferably 0.002% or below.

Al is an element not only acting as a deoxidizing agent, but also acting to form AlN by combining with N, and to refine the structure and improve toughness of the hot rolled wire rod. To make these actions be exerted, it is preferable to contain 0.0001% or above, more preferably 0.0002% or above, further more preferably 0.0003% or above. However, if excessively contained, hard oxide (Al₂O₃ or the like, for example) is formed in the hot rolled wire rod which becomes the cause of wire breakage in wire drawing. Therefore, Al is made 0.003% or below, preferably 0.002% or below, more preferably 0.001% or below.

O (oxygen) is an inevitable impurity element, and if O becomes excessive, coarse oxide-based inclusions are formed in the hot rolled wire rod which becomes the cause of wire breakage in wire drawing. Therefore, O is made 0.003% or below, preferably 0.0025% or below, more preferably 0.002% or below, further more preferably 0.0015% or below, most preferably 0.001% or below.

The hot rolled wire rod in accordance with the present invention contains the elements described above and the balance is iron and inevitable impurities.

As other elements, the hot rolled wire rod in accordance with the present invention may contain (1) high strengthening elements such as Cr, and (2) anti-corrosion property improve elements such as Cu.
(1) Cr is an element contributing to improving hardenability and increasing the strength of wire rod products. To exert these actions effectively, it is preferable to contain Cr by 0.01% or above, more preferably 0.02% or above, further more preferably 0.1% or above. However, if Cr is contained in excess, the tensile strength of the hot rolled wire rod becomes too high, super cooled structure is liable to be formed, and wire drawability deteriorates. Therefore, if present Cr is 0.5% or below, preferably 0.45% or below, more preferably 0.4% or below.
(2) Cu is an element contributing to not only inhibiting surface layer decarburization but also to improving anti-corrosion property of wire rod products. To exert such actions effectively, it is preferable to contain Cu by 0.01% or above, more preferably 0.05% or above, further more preferably 0.1% or above. However, if Cu is contained in excess, crack is generated in hot rolling, super cooled structure is formed, and wire drawability deteriorates. Therefore, if present Cu is 0.5% or below, preferably 0.45% or below, more preferably 0.4% or below.

In the hot rolled wire rod in accordance with the present invention, it is important that the chemical composition described above is contained, and, in addition, that tensile strength (TS) is 960 MPa or below and reduction of area (RA) is 40% or above. If tensile strength (TS) exceeds 960 MPa, working heat quantity generated in wire drawing increases, seizure occurs during wire drawing, thereby the life time of a dice is shortened and wire breakage occurs. On the other hand, if reduction of area (RA) is below 40%, cuppy break becomes liable to occur during wire drawing.

The tensile strength and the reduction of area of the hot rolled wire rod in accordance with the present invention are obtained by cutting test pieces for tensile test from the wire rod obtained by hot rolling, measuring tensile strength (TS) and reduction of area (RA) on a plurality of test pieces (number of the test pieces is 80, for example) according to ordinary methods, and averaging them. The strain rate in testing can be made 1.0×10⁻³*ₛ*⁻¹ to 3.5×10⁻³*ₛ*⁻¹.

The hot rolled wire rod in accordance with the present invention described above can be produced by appropriately controlling the hot rolling condition and the cooling condition after hot rolling. In other words, for the hot rolled wire rod in accordance with the present invention, the hot rolling condition and the cooling condition after hot rolling are to be controlled to follow the heat pattern exhibited in FIG. 1, and if
(a) a process for heating a billet satisfying the above composition at from 1,000 to 1,080 DEG C.,
(b) a process for hot rolling of the heated billet with the lowest temperature during rolling being made at from 820 to 920 DEG C.,
(c) a process for finish rolling of the wire rod obtained by the hot rolling at from 900 to 980 DEG C.,
(d) a process for winding the wire rod obtained by the finish rolling at from 880 to 940 DEG C.,
(e) a process for cooling the wound wire rod from the winding temperature to 800 DEG C. at average cooling rate (CR₁) of 10 DEG C./s or below,
(f) a process for cooling consecutively from 800 DEG C. to the temperature T₁ of 640-600 DEG C. at average cooling rate (CR₂) of 30 DEG C./s or above, and
(g) a process for heating the wire rod cooled to the temperature range of 640-600 DEG C. at a temperature T₂ of 680 DEG C. or below, wherein the temperature T₂ exceeds the temperature T₁ are performed in this order, the hot rolled wire rod in accordance with the present invention can be produced. The reasons such producing conditions were stipulated are as follows.

(a) If the heating temperature of the billet exceeds 1,080 DEG C., the tensile strength of the hot rolled wire rod increases, the reduction of area decreases, and wire drawability deteriorates. Therefore, in the present invention, the heating temperature of the billet is made 1,080 DEG C. or below. The lower limit of the heating temperature of the billet is approximately 1,000 DEG C. The preferable upper limit of the heating temperature of the billet is 1,060 DEG C. and the preferable lower limit is 1,020 DEG C.
(b) In hot rolling of the billet heated to the heating temperature described above, if the lowest temperature during rolling exceeds 920 DEG C., the tensile strength of the hot rolled wire rod increases, the reduction of area decreases, and wire drawability deteriorates. Therefore, according to the present invention, hot rolling is performed with the lowest temperature during rolling being made 920 DEG C. or below. The lower limit of the lowest temperature during hot rolling is approximately 820 DEG C. The preferable upper limit of the lowest temperature during hot rolling is 900 DEG C., more preferable upper limit is 880 DEG C., preferable lower limit is 840 DEG C., more preferable lower limit is 860 DEG C.
(c) If the finish rolling temperature of the wire rod obtained by hot rolling exceeds 980 DEG C., the tensile strength of the hot rolled wire rod increases, or the reduction of area decreases, and wire drawability deteriorates. Therefore, in the present invention, finish rolling is performed with the finish rolling temperature being made 980 DEG C. or below. The lower limit of the finish rolling temperature is 900 DEG C. Preferable upper limit of the finish rolling temperature is 960 DEG C.
(d) After performing finish rolling, the wire rod is wound in ring-shape onto a transport device such as a conveyor, but if winding temperature exceeds 940 DEG C., the tensile strength of the hot rolled wire rod increases, the reduction of area decreases, and wire drawability deteriorates. Therefore, in the present invention, winding is performed with the winding temperature being made 940 DEG C. or below. Preferable upper limit of the winding temperature is 920 DEG C., and more preferable upper limit is 910 DEG C. However, if the winding temperature is made too low, mechanical descaling property (MD property) deteriorates, therefore, the winding temperature is made 880 DEG C. or above. More preferable lower limit of the winding temperature is 890 DEG C., further more preferable lower limit is 900 DEG C. Also, the winding temperature can be adjusted by controlling the condition of water cooling performed after finish rolling.

In (e) and (f), it is important that two-step cooling is performed with the boundary of 800 DEG C. from the winding temperature to a temperature T₁ in the temperature range of 640-600 DEG C., more specifically, slow cooling in the range from the winding temperature to 800 DEG C., and quick cooling in the range from 800 DEG C. to the temperature T₁. The mechanism of improvement of wire drawability by decrease of the tensile strength and increase of the reduction of area of the hot rolled wire rod by combination of slow cooling and quick cooling has not been clarified, but can be presumed as below.

The present inventors consider that ferrite is formed by slow cooling in the range from the winding temperature to 800 DEG C., and metal structure is made finer by quick cooling in the range from 800 DEG C. to the temperature T₁, thereby the tensile strength of hot rolled wire rod decreases, the reduction of area increases, and wire drawability can be improved.
(e) If average cooling rate (CR₁) from the winding temperature to 800 DEG C. exceeds 10 DEG C./s, the tensile strength of the hot rolled wire rod increases and wire drawability deteriorates. Therefore, in the present invention, CR₁ is made 10 DEG C./s or below, preferably 9 DEG C./s or below, more preferably 8 DEG C./s or below. Lower limit of the average cooling rate (CR₁) is not limited particularly, but is, for example, 1 DEG C./s, preferably 2 DEG C./s.
(f) If average cooling rate (CR₂) from 800 DEG C. to the temperature T₁ is below 30 DEG C./s, metal structure does not become finer, therefore, the reduction of area of the hot rolled wire rod decreases and wire drawability deteriorates. Therefore, in the present invention, the average cooling rate (CR₂) is made 30 DEG C./s or above, preferably 33 DEG C./s or above, more preferably 35 DEG C./s or above. Upper limit of the average cooling rate (CR₂) is not limited particularly, but is, for example, 65 DEG C./s, preferably 60 DEG C./s.

Further, if the temperature T₁ exceeds 640 DEG C., the reduction of area of the hot rolled wire rod decreases, and if the temperature T₁ is below 600 DEG C., the tensile strength of the hot rolled wire rod increases, and wire drawability of the hot rolled wire rod deteriorates. Therefore, in the present invention, the ultimate temperature T₁ in cooling from 800 DEG C. is made 640-600 DEG C., preferably 638 DEG C. or below, more preferably 635 DEG C. or below. Also, it is preferably 605 DEG C. or above, more preferably 610 DEG C, or above.
(g) If heated after cooling to the temperature T₁, the tensile strength of the hot rolled wire rod can be decreased, however, if heated to above 680 DEG C., the reduction of area decreases and wire drawability deteriorates. Therefore, in the present invention, after cooled to the temperature T₁, the wire rod is heated to a temperature T₂ of 680 DEG C. or below, exceeding the temperature T₁. The temperature T₂ is preferably 675 DEG C. or below, more preferably 670 DEG C. or below. Further, if kept as it is at the temperature T₁ or consecutively cooled to the room temperature after cooled to the temperature T₁, the tensile strength of the hot rolled wire rod becomes too high and wire drawability deteriorates.

The hot rolled wire rod in accordance with the present invention thus obtained becomes excellent in wire drawability because the tensile strength becomes 960 MPa or below and the reduction of area becomes 40% or above. By performing wire drawing this hot rolled wire rod after descaling according to an ordinary method (mechanical descaling, acid washing treatment, or the like, for example), a wire rod with tensile strength level of 3,000 MPa level can be obtained.

Although the present invention will be described below in further detail by referring to the examples, the present invention is by no means to be limited by the examples below and can be implemented with appropriate modifications added within the scope adaptable to the purposes described above and below, and any of them is to be included within the technical range of the present invention.

The billets (steel kinds of A1-A32) of the composition exhibited in TABLE 1 below (balance is iron and inevitable impurities) were subjected to heating, hot rolling, winding and cooling according to the heat pattern exhibited in FIG. 1, and the hot rolled wire rods of 5.5 mm diameter were produced. TABLE 2 and TABLE 3 below exhibit; heating temperature, the lowest temperature during rolling, finish rolling temperature, winding temperature, average cooling rate from winding temperature to 800 DEG C. (CR₁), average cooling rate from 800 DEG C. to a temperature T₁ in the temperature range of 640-600 DEG C. (CR₂), temperature T₂ when heated from the temperature T₁, respectively.

The tensile property was evaluated on the hot rolled wire rods obtained. The evaluation of the tensile property was performed by preparing 8 test pieces for tensile test by dividing one ring (the length of one ring is approximately 4 m) of the hot rolled wire rod into 8 pieces, and by performing tensile tests using the test pieces for 10 rings (80 pieces in total). The strain rate in the tensile test was set at 1.0×10⁻³*ₛ*⁻¹ to 3.5×10⁻³*ₛ*⁻¹ and tensile strength (TS: MPa) and reduction of area (RA: %) were measured. Average of all test pieces are referred to as tensile strength (TS) and reduction of area (RA) respectively, and the results are exhibited in TABLE 4 and TABLE 5 below.

Also, the relation between tensile strength (TS) and reduction of area (RA) is exhibited in FIG. 2. ○ in FIG. 2 exhibits the results of Nos.1-5, No.8, Nos.10-14, No.21, Nos.26-33, Nos.38-40, No.46, No.47, and Nos.53-55. × in FIG. 2 exhibits the results of No.6, No.7, No.9, No.15, Nos.22-25, Nos.34-37, Nos.41-45, Nos.49-52, and Nos.56-60.

Then, wire drawability of the hot rolled wire rods obtained was evaluated. After descaling the 5.5 mm diameter hot rolled wire rod, dry drawing was performed so that the final wire diameter becomes 0.9 mm using a continuous drawing machine, and wire drawability was evaluated based on whether wire breakage had occurred or not in wire drawing and the life time of the dice.

The wire drawing conditions were as described below, and 2 tons for each hot rolled wire rod were used for the test. Whether or not wire breakage had occurred was visually confirmed. The life time of the dice was evaluated according to the criteria described below by visually observing the dice after drawing. The results are exhibited in TABLE 4 and TABLE 5 below.

### [Condition of Drawing]

| | |
|---|---|
| Descaling: | Mechanical descaling (MD) |
| Number of dice: | 18 pieces |
| Final drawing speed: | 1,000 m/min (1,100 m/min only |
| when wire breakage did not occur at 1,000 m/min) | |
| Intermediate heat treatment:None | |

### [Evaluation Criteria of Life Time of Dice]

○ (passed): The case wherein replacement of the dice for breakage and wear of the dice was not necessary.
△ (Failed): The case wherein although breakage of the dice did not occur, replacement of the dice became necessary after wire drawing because of the wear of the dice.
× (Failed): The case wherein the dice was broken during wire drawing.
- (Failed): The case wherein the life time of the dice could not be evaluated because of wire breakage during wire drawing.

In the present invention, in the case wherein wire breakage did not occur and the life time of the dice passed in the evaluation when the final drawing speed was made 1,000 m/min, wire drawability was judged to be excellent, and in the case wherein wire breakage did not occur and the life time of the dice passed in the evaluation when the final drawing speed was made 1,100 m/min, wire drawability was judged to be particularly excellent.

Based on FIG. 2, following analysis is possible. In the example wherein the conditions stipulated in the present invention were satisfied (○ mark in FIG. 2), wire drawability could be improved. On the other hand, in the example wherein the conditions stipulated in the present invention were not satisfied (× mark in FIG. 2), if the tensile strength (TS) of the hot rolled wire rod had increased to exceed 960 MPa, seizure occurred in wire drawing and wire breakage occurred. Also, the life time of the dice was shortened. Further, if the reduction of area (RA) of the hot rolled wire rod had been below 40%, wire breakage occurred during wire drawing.

From TABLE 1-TABLE 5 below, following analysis is possible. In No.6 and No.56, because the cooling speed from winding temperature to 800 DEG C. had not been appropriately controlled, tensile strength increased and wire drawability could not be improved. In No.7, because the cooling speed from 800 DEG C. to the temperature T₁ had not been appropriately controlled, the reduction of area decreased and wire drawability could not be improved. In No.9, because the cooling speed from 800 DEG C. to the temperature T₁ had not been appropriately controlled, the reduction of area decreased. Further, because cooled to room temperature after maintained at the constant temperature for 15 seconds after cooled to 610 DEG C. (temperature T₁) after finish rolling, the tensile strength increased. Therefore, wire drawability could not be improved.

In Nos.15-20, No.48, No.49, No.52, No.59 and No.60, because the composition of the hot rolled wire rod had been deviated from the range the present invention had stipulated, wire drawability could not be improved. Particularly in No.59 and No.60 which are the examples wherein C had been contained by 0.80% or above, even if the cooling speed CR₁ and the cooling speed CR₂ had been appropriately controlled, the tensile strength increased, the reduction of area decreased, and wire drawability could not be improved.

In No.50, because Cu had been contained in excess, the tensile strength increased, and wire drawability could not be improved. In No.51, because Cr had been contained in excess, the tensile strength increased, the reduction of area decreased, and wire drawability could not be improved.

In No.22 and No.42, because the wire rod had been consecutively cooled to the room temperature after cooling from 800 DEG C. to the temperature T₁, the tensile strength increased, and wire drawability could not be improved. In No.23 and No.43, because the temperature T₁ had been too low, the tensile strength increased, and wire drawability could not be improved. In No.25 and No.44, because the temperature T₁ had been too high, the reduction of area decreased, and wire drawability could not be improved. In No.24 and No.45, because the heating temperature T₂ had been too high, the reduction of area decreased, and wire drawability could not be improved.

In No.34, because 2 stage cooling had not been adopted for the range from the winding temperature to the temperature T₁ but had been continually cooled, the tensile strength increased, the reduction of area decreased, and wire drawability could not be improved. In No.35, the heating temperature had been too high, In No.36, the lowest rolling temperature had been too high, and in No.37, the finish rolling temperature had been too high, therefore the tensile strength increased, the reduction of area decreased, and wire drawability could not be improved in all these examples.

In No.39 and No.40, which are examples for reference, because the winding temperature had been slightly low, MD property deteriorated a little. In No.41, because the winding temperature had been too high, the tensile strength increased, and wire drawability could not be improved.

In No.57, because the cooling speed from 800 DEG C. to the temperature T₁ had not been appropriately controlled, the reduction of area decreased, and wire drawability could not be improved. In No.58, because the cooling speed from 800 DEG C. to the temperature T₁ had not been appropriately controlled, the reduction of area decreased. Also, because the temperature T₁ had been too low, the tensile strength increased. Therefore, wire drawability could not be improved.

**[TABLE 1]**

| Steel kind | Composition (mass%) | | | | | | | | | |
|---|---|---|---|---|---|---|---|---|---|---|
| | C | Si | Mn | P | S | Cu | Cr | Al | N | O |
| A1 | 0.65 | 0.47 | 0.58 | 0.007 | 0.007 | 0.42 | 0.45 | 0.0004 | 0.0034 | 0.0014 |
| A2 | 0.70 | 0.17 | 0.57 | 0.006 | 0.003 | - | - | 0.0010 | 0.0038 | 0.0011 |
| A3 | 0.71 | 0.10 | 0.46 | 0.002 | 0.010 | 0.10 | 0.28 | 0.0005 | 0.0025 | 0.0011 |
| A4 | 0.71 | 0.30 | 0.36 | 0.011 | 0.008 | - | 0.33 | 0.0006 | 0.0019 | 0.0015 |
| A5 | 0.71 | 0.22 | 0.49 | 0.008 | 0.003 | - | - | 0.0003 | 0.0026 | 0.0012 |
| A6 | 0.71 | 0.14 | 0.51 | 0.011 | 0.007 | - | - | 0.0010 | 0.0035 | 0.0014 |
| A7 | 0.71 | 0.28 | 0.47 | 0.004 | 0.010 | - | - | 0.0007 | 0.0039 | 0.0012 |
| A8 | 0.71 | 0.14 | 0.50 | 0.014 | 0.013 | - | - | 0.0008 | 0.0019 | 0.0012 |
| A9 | 0.71 | 0.83 | 0.50 | 0.005 | 0.004 | - | - | 0.0008 | 0.0040 | 0.0011 |
| A10 | 0.71 | 0.22 | 0.02 | 0.005 | 0.012 | - | - | 0.0005 | 0.0039 | 0.0009 |
| A11 | 0.71 | 0.23 | 0.48 | 0.020 | 0.005 | - | - | 0.0008 | 0.0023 | 0.0009 |
| A12 | 0.71 | 0.17 | 0.46 | 0.014 | 0.018 | - | - | 0.0003 | 0.0033 | 0.0014 |
| A13 | 0.71 | 0.25 | 0.48 | 0.008 | 0.009 | - | - | 0.0332 | 0.0030 | 0.0008 |
| A14 | 0.71 | 0.21 | 0.50 | 0.004 | 0.010 | - | - | 0.0006 | 0.0025 | 0.0040 |
| A15 | 0.72 | 0.20 | 0.48 | 0.014 | 0.011 | 0.01 | - | 0.0004 | 0.0016 | 0.0014 |
| A16 | 0.72 | 0.16 | 0.55 | 0.006 | 0.007 | - | 0.02 | 0.0007 | 0.0020 | 0.0014 |
| A17 | 0.72 | 0.29 | 0.48 | 0.009 | 0.004 | - | - | 0.0004 | 0.0030 | 0.0008 |
| A18 | 0.72 | 0.32 | 0.27 | 0.015 | 0.004 | - | - | 0.0008 | 0.0027 | 0.0013 |
| A19 | 0.72 | 0.22 | 0.47 | 0.011 | 0.003 | - | - | 0.0006 | 0.0027 | 0.0015 |
| A20 | 0.72 | 0.22 | 0.45 | 0.008 | 0.004 | - | - | 0.0004 | 0.0025 | 0.0010 |
| A21 | 0.72 | 0.16 | 0.55 | 0.004 | 0.009 | 0.01 | 0.01 | 0.0007 | 0.0015 | 0.0010 |
| A22 | 0.72 | 0.10 | 0.52 | 0.014 | 0.003 | - | - | 0.0009 | 0.0018 | 0.0009 |
| A23 | 0.72 | 0.03 | 0.46 | 0.005 | 0.007 | - | - | 0.0247 | 0.0016 | 0.0010 |
| A24 | 0.72 | 0.21 | 0.77 | 0.004 | 0.006 | - | - | 0.0002 | 0.0037 | 0.0010 |
| A25 | 0.72 | 0.25 | 0.47 | 0.010 | 0.007 | 0.62 | - | 0.0004 | 0.0015 | 0.0014 |
| A26 | 0.72 | 0.23 | 0.54 | 0.012 | 0.010 | - | 0.70 | 0.0005 | 0.0038 | 0.0010 |
| A27 | 0.72 | 0.20 | 0.54 | 0.012 | 0.009 | - | - | 0.0003 | 0.0051 | 0.0012 |
| A28 | 0.74 | 0.14 | 0.54 | 0.007 | 0.010 | - | - | 0.0005 | 0.0020 | 0.0014 |
| A29 | 0.74 | 0.19 | 0.14 | 0.004 | 0.003 | - | - | 0.0002 | 0.0015 | 0.0015 |
| A30 | 0.75 | 0.24 | 0.22 | 0.013 | 0.008 | 0.15 | 0.20 | 0.0004 | 0.0032 | 0.0012 |
| A31 | 0.80 | 0.27 | 0.55 | 0.009 | 0.006 | - | - | 0.0007 | 0.0036 | 0.0013 |
| A32 | 0.83 | 0.23 | 0.45 | 0.012 | 0.010 | - | - | 0.0009 | 0.0032 | 0.0012 |

**[TABLE 2]**

| No. | Steel kind | Heating temp. (DEG C.) | Lowest rolling temp. | Finish rolling temp. | Winding temp. | Cooling rate | | Temp. | | Remarks |
|---|---|---|---|---|---|---|---|---|---|---|
| | | | (DEG C.) | (DEG C.) | (DEG C.) | CR₁ (DEG C./s) | CR₂ (DEG C./s) | T₁ (DEG C.) | T₂ (DEG C.) | |
| 1 | A1 | 1038 | 898 | 947 | 920 | 4 | 48 | 624 | 680 | |
| 2 | A2 | 1059 | 879 | 933 | 909 | 4 | 48 | 600 | 653 | |
| 3 | A3 | 1055 | 889 | 944 | 904 | 4 | 43 | 614 | 652 | |
| 4 | A4 | 1055 | 900 | 950 | 937 | 5 | 43 | 630 | 671 | |
| 5 | A5 | 1056 | 880 | 931 | 891 | 4 | 58 | 610 | 627 | |
| 6 | A5 | 1049 | 873 | 923 | 904 | 17 | 39 | 602 | 630 | |
| 7 | A5 | 1043 | 891 | 946 | 900 | 5 | 14 | 638 | 641 | |
| 8 | A5 | 1036 | 898 | 940 | 906 | 4 | 55 | 614 | 668 | |
| 9 | A5 | 1055 | 878 | 931 | 902 | 7 | 24 | 610 | - | Maintained at constant temp. |
| 10 | A6 | 1043 | 881 | 935 | 899 | 3 | 35 | 637 | 649 | |
| 11 | A6 | 1040 | 874 | 930 | 900 | 7 | 41 | 627 | 655 | |
| 12 | A6 | 1030 | 870 | 922 | 900 | 6 | 43 | 625 | 662 | |
| 13 | A7 | 1047 | 878 | 933 | 924 | 3 | 32 | 626 | 648 | |
| 14 | A8 | 1052 | 875 | 929 | 901 | 3 | 43 | 611 | 651 | |
| 15 | A9 | 1048 | 899 | 942 | 894 | 6 | 36 | 634 | 655 | |
| 16 | A10 | 1048 | 886 | 939 | 909 | 8 | 47 | 632 | 664 | |
| 17 | A11 | 1033 | 896 | 946 | 908 | 4 | 35 | 618 | 624 | |
| 18 | A12 | 1055 | 891 | 942 | 910 | 7 | 34 | 625 | 634 | |
| 19 | A13 | 1037 | 881 | 936 | 892 | 7 | 48 | 621 | 660 | |
| 20 | A14 | 1031 | 894 | 947 | 890 | 8 | 49 | 613 | 659 | |
| 21 | A15 | 1050 | 885 | 936 | 903 | 6 | 43 | 613 | 652 | |
| 22 | A15 | 1055 | 893 | 946 | 896 | 7 | 31 | 627 | - | Continuous cooling |
| 23 | A15 | 1046 | 876 | 928 | 895 | 4 | 32 | 588 | 605 | |
| 24 | A15 | 1055 | 890 | 942 | 903 | 8 | 33 | 639 | 684 | |
| 25 | A15 | 1046 | 892 | 944 | 892 | 3 | 34 | 655 | 678 | |
| 26 | A16 | 1057 | 876 | 928 | 895 | 4 | 37 | 623 | 670 | |
| 27 | A16 | 1055 | 870 | 924 | 901 | 3 | 42 | 627 | 668 | |
| 28 | A16 | 1054 | 871 | 924 | 903 | 4 | 53 | 612 | 660 | |
| 29 | A17 | 1041 | 871 | 922 | 897 | 6 | 43 | 632 | 660 | |
| 30 | A17 | 1040 | 876 | 926 | 899 | 4 | 37 | 635 | 662 | |

**[TABLE 3]**

| No. | Steel kind | Heating temp. (DEG C.) | Lowest rolling temp. | Finish rolling temp. | Winding temp. | Cooling rate | | Temp. | | Remarks |
|---|---|---|---|---|---|---|---|---|---|---|
| | | | | | | CR₁ | CR₂ | T₁ | T₂ | |
| | | | (DEG C.) | (DEG C.) | (DEG C.) | (DEG C./s) | (DEG C./s) | (DEG C.) | (DEG C.) | |
| 31 | A17 | 1035 | 870 | 920 | 902 | 3 | 31 | 638 | 657 | |
| 32 | A18 | 1042 | 900 | 937 | 893 | 7 | 32 | 640 | 671 | |
| 33 | A19 | 1036 | 873 | 924 | 907 | 9 | 38 | 634 | 665 | |
| 34 | A19 | 1045 | 882 | 939 | 907 | 23 | 23 | 617 | 639 | One step cooling |
| 35 | A19 | 1091 | 898 | 947 | 891 | 5 | 50 | 630 | 666 | |
| 36 | A19 | 1059 | 925 | 950 | 905 | 7 | 49 | 637 | 638 | |
| 37 | A19 | 1057 | 900 | 988 | 910 | 4 | 48 | 625 | 636 | |
| 38 | A20 | 1032 | 889 | 942 | 909 | 6 | 45 | 638 | 662 | |
| 39 | A20 | 1041 | 896 | 946 | 872 | 3 | 31 | 636 | 670 | MD property slightly bad |
| 40 | A20 | 1057 | 888 | 930 | 843 | 3 | 30 | 623 | 669 | MD property slightly bad |
| 41 | A20 | 1057 | 892 | 950 | 945 | 7 | 42 | 615 | 635 | |
| 42 | A20 | 1045 | 895 | 945 | 893 | 5 | 32 | 630 | - | Continuous cooling |
| 43 | A20 | 1058 | 871 | 923 | 898 | 6 | 39 | 588 | 614 | |
| 44 | A20 | 1031 | 871 | 923 | 897 | 7 | 50 | 647 | 661 | |
| 45 | A20 | 1043 | 884 | 936 | 905 | 6 | 32 | 638 | 685 | |
| 46 | A21 | 1052 | 898 | 948 | 900 | 6 | 49 | 620 | 663 | |
| 47 | A22 | 1052 | 891 | 941 | 907 | 10 | 30 | 631 | 671 | |
| 48 | A23 | 1039 | 891 | 943 | 901 | 7 | 37 | 615 | 621 | |
| 49 | A24 | 1052 | 881 | 935 | 893 | 4 | 48 | 616 | 626 | |
| 50 | A25 | 1049 | 870 | 925 | 904 | 6 | 48 | 618 | 624 | |
| 51 | A26 | 1044 | 873 | 925 | 903 | 4 | 31 | 613 | 652 | |
| 52 | A27 | 1033 | 893 | 947 | 891 | 6 | 42 | 631 | 634 | |
| 53 | A28 | 1045 | 895 | 946 | 894 | 3 | 46 | 622 | 670 | |
| 54 | A29 | 1050 | 898 | 950 | 894 | 3 | 42 | 636 | 662 | |
| 55 | A30 | 1040 | 897 | 949 | 901 | 4 | 30 | 636 | 678 | |
| 56 | A30 | 1045 | 889 | 942 | 910 | 15 | 44 | 605 | 646 | |
| 57 | A30 | 1056 | 883 | 934 | 905 | 8 | 25 | 637 | 669 | |
| 58 | A30 | 1050 | 887 | 941 | 894 | 8 | 26 | 591 | 608 | |
| 59 | A31 | 1049 | 899 | 950 | 908 | 6 | 50 | 639 | 658 | |
| 60 | A32 | 1031 | 890 | 944 | 899 | 8 | 44 | 625 | 636 | |

**[TABLE 4]**

| No. | Tensile strength | Reduction of area | Wire drawing | | | |
|---|---|---|---|---|---|---|
| | TS | RA | 1,000m/min | | 1,100m/min | |
| | (MPa) | (%) | Wire breakage | Life of dice | Wire breakage | Life of dice |
| 1 | 953 | 49 | No | ○ | No | ○ |
| 2 | 952 | 47 | No | ○ | No | ○ |
| 3 | 957 | 45 | No | ○ | No | ○ |
| 4 | 941 | 43 | No | ○ | No | ○ |
| 5 | 951 | 44 | No . | ○ | No | ○ |
| 6 | 967 | 42 | No | × | Yes | - |
| 7 | 957 | 38 | Yes | - | - | - |
| 8 | 937 | 40 | No | ○ | No | ○ |
| 9 | 977 | 37 | Yes | - | - | - |
| 10 | 951 | 44 | No | ○ | No | ○ |
| 11 | 945 | 42 | No | ○ | No | ○ |
| 12 | 940 | 41 | No | ○ | No | ○ |
| 13 | 950 | 44 | No | ○ | No | ○ |
| 14 | 949 | 44 | No | ○ | No | ○ |
| 15 | 980 | 42 | Yes | - | - | - |
| 16 | 924 | 43 | Yes | - | - | - |
| 17 | 949 | 44 | Yes | - | - | - |
| 18 | 944 | 44 | Yes | - | - | - |
| 19 | 950 | 44 | Yes | - | - | - |
| 20 | 952 | 44 | Yes | - | - | - |
| 21 | 954 | 43 | No | ○ | No | ○ |
| 22 | 974 | 42 | No | × | Yes | - |
| 23 | 991 | 44 | Yes | - | - | - |
| 24 | 940 | 37 | Yes | - | - | - |
| 25 | 938 | 33 | Yes | - | - | - |
| 26 | 945 | 42 | No | ○ | No | ○ |
| 27 | 945 | 44 | No | ○ | No | ○ |
| 28 | 940 | 42 | No | ○ | No | ○ |
| 29 | 951 | 43 | No | ○ | No | ○ |
| 30 | 949 | 41 | No | ○ | No | ○ |

**[TABLE 5]**

| No. | Tensile strength | Reduction of area | Wire drawling | | | |
|---|---|---|---|---|---|---|
| | TS | RA | 1,000m/min | | 1,100m/min | |
| | (MPa) | (%) | Wire breakage | Life of dice | Wire breakage | Life of dice |
| 31 | 946 | 41 | No | ○ | No | ○ |
| 32 | 928 | 44 | No | ○ | No | ○ |
| 33 | 952 | 43 | No | ○ | No | ○ |
| 34 | 980 | 37 | Yes | - | - | - |
| 35 | 1008 | 35 | Yes | - | - | - |
| 36 | 1012 | 36 | Yes | - | - | - |
| 37 | 1020 | 37 | Yes | - | - | - |
| 38 | 954 | 43 | No | ○ | No | ○ |
| 39 | 942 | 45 | No | ○ | No | Δ |
| 40 | 938 | 47 | No | ○ | No | Δ |
| 41 | 989 | 42 | Yes | - | - | - |
| 42 | 997 | 40 | Yes | - | - | - |
| 43 | 1021 | 42 | Yes | - | - | - |
| 44 | 952 | 37 | Yes | - | - | - |
| 45 | 935 | 34 | Yes | - | - | - |
| 46 | 953 | 42 | No | ○ | No | ○ |
| 47 | 957 | 43 | No | ○ | No | ○ |
| 48 | 949 | 44 | Yes | - | - | - |
| 49 | 1011 | 40 | Yes | - | - | - |
| 50 | 997 | 40 | Yes | - | - | - |
| 51 | 1119 | 33 | Yes | - | - | - |
| 52 | 1010 | 42 | Yes | - | - | - |
| 53 | 956 | 41 | No | ○ | No | ○ |
| 54 | 948 | 46 | No | ○ | No | ○ |
| 55 | 960 | 42 | No | ○ | No | ○ |
| 56 | 1012 | 42 | Yes | - | - | - |
| 57 | 957 | 34 | Yes | - | - | - |
| 58 | 1028 | 38 | Yes | - | - | - |
| 59 | 1059 | 37 | Yes | - | - | - |
| 60 | 1071 | 36 | Yes | - | - | - |

## Claims

1. A wire rod excellent in wire drawability consisting of,
C: 0.65-0.75%,
Si: 0.1-0.5%.
Mn: 0.1-0.6%,
P: 0.015% or below, not including 0%,
S: 0.015% or below, not including 0%,
N: 0.004% or below, not including 0%,
Al: 0.003% or below, not including 0%,
O: 0.003% or below, not including 0%,
optionally Cr: 0.5% or below, not including 0%,
optionally Cu: 0.5% or below, not including 0%, and
the balance being iron and inevitable impurities,
wherein % indicates mass% with regard to the composition,
wherein tensile strength (TS) is 960 MPa or below, and reduction of area (RA) is 40% or above, obtainable by a method comprising
a process for heating a billet satisfying the above composition at from 1,000 to 1,080 DEG C.,
a process for hot rolling of the heated billet with the lowest temperature during rolling being made at from 820 to 920 DEG C.,
a process for finish rolling of the wire rod obtained by the hot rolling at from 900 to 980 DEG C.,
a process for winding the wire rod obtained by the finish rolling at from 880 to 940 DEG C.,
a process for cooling the wound wire rod from the winding temperature to 800 DEG C. at average cooling rate (CR₁) of 10 DEG C./s or below,
a process for cooling consecutively from 800 DEG C. to the temperature T₁ of 640-600 DEG C. at average cooling rate (CR₂) of 30 DEG C./s or above, and
a process for heating the wire rod cooled to the temperature T₁ at a temperature T₂ of 680 DEG C. or below, wherein the temperature T₂ exceeds the temperature T₁.

2. A method for producing a wire rod excellent in wire drawability comprising
a process for heating a billet satisfying the composition as set forth in Claim 1 at from 1,000 to 1,080 DEG C.,
a process for hot rolling of the heated billet with the lowest temperature during rolling being made at from 820 to 920 DEG C.,
a process for finish rolling of the wire rod obtained by the hot rolling at from 900 to 980 DEG C.,
a process for winding the wire rod obtained by the finish rolling at from 880 to 940 DEG C.,
a process for cooling the wound wire rod from the winding temperature to 800 DEG C. at average cooling rate (CR₁) of 10 DEG C./s or below,
a process for cooling consecutively from 800 DEG C. to the temperature T₁ of 640-600 DEG C. at average cooling rate (CR₂) of 30 DEG C./s or above, and
a process for heating the wire rod cooled to the temperature T₁ at a temperature T₂ of 680 DEG C. or below, wherein the temperature T₂ exceeds the temperature T₁.

## Patentansprüche

1. Walzdraht mit hervorragender Drahtziehfähigkeit, bestehend aus
C: 0,65 - 0,75%,
Si: 0,1 - 0,5%.
Mn: 0,1 - 0,6%,
P: 0,015% oder niedriger, 0% nicht eingeschlossen,
S: 0,015% oder niedriger, 0% nicht eingeschlossen,
N: 0,004% oder niedriger, 0% nicht eingeschlossen,
Al: 0,003% oder niedriger, 0% nicht eingeschlossen,
O: 0,003% oder niedriger, 0% nicht eingeschlossen,
gegebenenfalls Cr: 0,5% oder niedriger, 0% nicht eingeschlossen,
gegebenenfalls Cu: 0,5% oder niedriger, 0% nicht eingeschlossen, und wobei der Rest Eisen und unvermeidbare Verunreinigungen ist,
wobei % Masse-% in Bezug auf die Zusammensetzung bedeutet,
wobei die Zugfestigkeit (TS) 960 MPa oder niedriger beträgt und die Brucheinschnürung (RA) 40% oder höher beträgt, erhältlich durch ein Verfahren, umfassend
ein Verfahren zum Erwärmen eines Stranges, der der vorstehenden Zusammensetzung genügt, auf 1000 bis 1080°C,
ein Verfahren zum Warmwalzen des erwärmten Stranges, wobei die niedrigste Temperatur während des Walzens auf 820 bis 920°C eingestellt ist,
ein Verfahren zum Fertigwalzen des durch das Warmwalzen erhaltenen Walzdrahtes bei 900 bis 980°C,
ein Verfahren zum Wickeln des durch das Fertigwalzen erhaltenen Walzdrahtes bei 880 bis 940°C,
ein Verfahren zum Kühlen des gewickelten Walzdrahtes von der Wickeltemperatur bis 800°C bei einer mittleren Kühlrate (CR₁) von 10°C/s oder niedriger,
ein Verfahren zum nachfolgenden Kühlen von 800°C bis zu der Temperatur T₁ von 640 - 600°C bei einer mittleren Kühlrate (CR₂) von 30°C/s oder höher, und
ein Verfahren zum Erwärmen des auf die Temperatur T₁ gekühlten Walzdrahtes auf eine Temperatur T₂ von 680°C oder niedriger, wobei die Temperatur T₂ größer ist als die Temperatur T₁.

2. Verfahren zur Herstellung eines Walzdraht mit hervorragender Drahtziehfähigkeit, umfassend
ein Verfahren zum Erwärmen eines Stranges, der der Zusammensetzung, wie im Anspruch 1 definiert, genügt, auf 1000 bis 1080°C,
ein Verfahren zum Warmwalzen des erwärmten Stranges, wobei die niedrigste Temperatur während des Walzens auf 820 bis 920°C eingestellt ist,
ein Verfahren zum Fertigwalzen des durch das Warmwalzen erhaltenen Walzdrahtes bei 900 bis 980°C,
ein Verfahren zum Wickeln des durch das Fertigwalzen erhaltenen Walzdrahtes bei 880 bis 940°C,
ein Verfahren zum Kühlen des gewickelten Walzdrahtes von der Wickeltemperatur bis 800°C bei einer mittleren Kühlrate (CR₁) von 10°C/s oder niedriger,
ein Verfahren zum nachfolgenden Kühlen von 800°C bis zu der Temperatur T₁ von 640 - 600°C bei einer mittleren Kühlrate (CR₂) von 30°C/s oder höher, und
ein Verfahren zum Erwärmen des auf die Temperatur T₁ gekühlten Walzdrahtes auf eine Temperatur T₂ von 680°C oder niedriger, wobei die Temperatur T₂ größer ist als die Temperatur T₁.

## Revendications

1. Fil-machine présentant une excellente aptitude à l'étirage constitué de
C: 0,65-0,75%,
Si: 0,1-0,5%.
Mn: 0,1-0,6%,
P: 0,015% ou moins, 0% n'est pas compris,
S: 0,015% ou moins, 0% n'est pas compris,
N: 0,004% ou moins, 0% n'est pas compris,
Al: 0,003% ou moins, 0% n'est pas compris,
O: 0,003% ou moins, 0% n'est pas compris,
éventuellement Cr: 0,5% ou moins, 0% n'est pas compris,
éventuellement Cu: 0,5% ou moins, 0% n'est pas compris, et
le reste étant du fer et des impuretés inévitables,
où % indique % en masse par rapport à la composition,
où la résistance à la traction (TS) est de 960 MPa ou moins, et la réduction de section (RA) est de 40% ou plus, pouvant être obtenues par un procédé comprenant
un processus de chauffage d'une billette satisfaisant la composition ci-dessus à une température allant de 1000 à 1080°C,
un processus de laminage à chaud de la billette chauffée avec la température la plus basse pendant le laminage étant réalisé à une température allant de 820 à 920°C,
un processus de laminage de finition du fil-machine obtenu par le laminage à chaud à une température allant de 900 à 980°C,
un processus d'enroulement du fil-machine obtenu par le laminage de finition à une température allant de 880 à 940°C,
un processus de refroidissement du fil-machine enroulé à partir de la température d'enroulement jusqu'à 800°C à une vitesse de refroidissement moyenne (CR₁) de 10°C/s ou moins,
un processus de refroidissement de façon consécutive à partir de 800°C jusqu'à la température T₁ de 640-600°C à une vitesse de refroidissement moyenne (CR₂) de 30°C/s ou plus, et
un processus de chauffage du fil-machine refroidi jusqu'à la température T₁ à une température T₂ de 680°C ou moins, où la température T₂ dépasse la température T₁.

2. Procédé de production d'un fil-machine présentant une excellente aptitude à l'étirage comprenant
un processus de chauffage d'une billette satisfaisant la composition selon la revendication 1 à une température allant de 1000 à 1080°C,
un processus de laminage à chaud de la billette chauffée avec la température la plus basse pendant le laminage étant réalisé à une température allant de 820 à 920°C,
un processus de laminage de finition du fil-machine obtenu par le laminage à chaud à une température allant de 900 à 980°C,
un processus d'enroulement du fil-machine obtenu par le laminage de finition à une température allant de 880 à 940°C,
un processus de refroidissement du fil-machine enroulé à partir de la température d'enroulement jusqu'à 800°C à une vitesse de refroidissement moyenne (CR₁) de 10°C/s ou moins,
un processus de refroidissement de façon consécutive à partir de 800°C jusqu'à la température T₁ de 640-600°C à une vitesse de refroidissement moyenne (CR₂) de 30°C/s ou plus, et
un processus de chauffage du fil-machine refroidi jusqu'à la température T₁ à une température T₂ de 680°C ou moins, où la température T₂ dépasse la température T₁.
